

# UNITED STATES PATENT OFFICE.

GEORGE ROCKER, OF WILMINGTON, DELAWARE, ASSIGNOR TO E. I. DU PONT DE NEMOURS & COMPANY, OF WILMINGTON, DELAWARE, A CORPORATION OF DELAWARE.

## METHOD OF CONTROLLING THE STABILIZER CONTENT OF CELLULOSIC COLLOIDS.

1,424,212.

Specification of Letters Patent.

Patented Aug. 1, 1922.

No Drawing.

Application filed December 17, 1920. Serial No. 431,396.

To all whom it may concern:

Be it known that I, GEORGE ROCKER, a citizen of the United States, and a resident of Wilmington, in the county of New Castle

5 and State of Delaware, have invented a certain new and useful Method of Controlling the Stabilizer Content of Cellulosic Colloids, of which the following is a specification.

10 This invention relates to the treatment of cellulosic colloids and has more particular reference to a method of treating cellulosic colloids to control the stabilizer content thereof, either to add stabilizer to the colloid being treated, or to overcome and offset extraction of stabilizer from the colloid during treatment with a solvent for the stabilizer. In this latter mentioned aspect the method finds a particularly advantageous

15 application when used in connection with a method whereby ethyl ether used for colloiding is extracted from nitrocellulose powder by washing with ethyl alcohol, the method of this invention providing for the 20 retention in the powder, during the said washing, of the desired and previously introduced stabilizer, despite the fact that alcohol is a solvent for the stabilizer, e. g. diphenylamine. Since the method finds advantageous application in the art of manufacturing nitrocellulose powder I describe it with more particular reference to that art, but do not confine it thereto, nor to the treatment of nitrocellulose colloids.

25 I have discovered that a stabilizer, for example, diphenylamine, can be added to nitrocellulose powder by treating the powder with a solution of the stabilizer, as, for example, an ethyl alcohol solution, and have 30 also discovered that the stabilizer content of powder may be held constant during washing with a volatile solvent for the stabilizer, e. g. ethyl alcohol, provided stabilizer be added to the solvent in an amount sufficient 35 to give equilibrium between the stabilizer in the powder and that in the solvent. The present method is based upon these discoveries.

40 In working with diphenylamine as a stabilizer various strengths of alcohol may be used. As I prefer to use 60% or 80% of alcohol by volume (alcohol-water solution) I refer more particularly to these strengths and confine my examples, etc., to them; but

as will be evident, the method may be carried out with other strengths of alcohol, and, indeed, with other stabilizers, for example dinitrotoluol, and other solvents.

45 With 60% alcohol, my experiments show that for either adding diphenylamine to the powder, or for holding in the powder during the washing, the diphenylamine previously added thereto, the necessary percentage ( $y$ ) of diphenylamine in the alcohol is given by the formula:

$$y = \frac{X - B}{4.5};$$

50 where  $X$  = % of diphenylamine desired in the finished powder, and  $B$  = % of diphenylamine already in the powder, this latter percentage being on a "finished powder" basis, i. e.

$$\frac{\text{weight of diphenylamine}}{\text{weight finished powder}} \times 100; \quad 75$$

55 but  $B$ , for any values above .37, is to be taken as constant, .37, since I have found that practically speaking, diphenylamine-free 60% alcohol will, by extraction, reduce 60 greater than .37% of diphenylamine in the powder down to .37%, but will not reduce it below that percentage. For 80% alcohol and diphenylamine the formula corresponding to that given for 60% alcohol is  $85$

$$y = \frac{X - B}{2.5};$$

65 and  $B$ , for any values above .25, is to be taken as a constant, .25, since I have found 70 that, for practical purposes, diphenylamine-free 80% alcohol will, by extraction, reduce greater than .25% of diphenylamine in the powder down to .25%, but will not reduce it below that percent.  $75$

75 As will appear from the specific examples given hereinafter, it is not generally necessary that the calculated amount be exactly adhered to, since small departures therefrom are permissible in practical work.  $80$

80 In treating powder to add thereto sufficient diphenylamine to give a desired specified percentage it is desirable to wash the powder, with the aid of any suitable device having provisions for continuous inflow and outflow, with a flow of alcohol containing 105 the calculated percentage of diphenylamine corresponding to the said "specified" per-

centage in the powder, until test of the off-flowing alcohol shows that no diphenylamine has been lost by the alcohol in its passage through the powder, continuously introduced "fresh" alcohol, containing the calculated percentage of diphenylamine, being of course used for the washing. With the alcohol losing no diphenylamine in its passage, of course no more diphenylamine is being added to the powder; but alcohol containing the calculated percentage of diphenylamine will add diphenylamine to the powder up to the "specified" percentage, so that, with the condition of no-diphenylamine-lost reached, the specified percentage of diphenylamine has been added; further washing, with alcohol of the calculated percentage has no effect on the specified percentage of diphenylamine in the powder, as alcohol containing the calculated percentage of diphenylamine gives equilibrium at the specified percentage.

The diphenylamine having been added to the powder, the alcohol is next removed from the powder, this being preferably done by first draining the alcohol from the powder and then washing with a liquid with which the alcohol is miscible but which is not a solvent for diphenylamine, e. g. water. As will be understood by those skilled in the art there should be used, of the solution of calculated diphenylamine strength, a quantity in excess of that containing merely the total weight of diphenylamine that it is desired to add to the batch of powder since the entire content of diphenylamine in the solution will not be transferred to the powder; the excess desirable will of course vary with the particular powder being treated. As examples of increasing the diphenylamine content of powder I have, using 60% alcohol containing 6 pounds of diphenylamine per 10,000 pounds of solution, raised the diphenylamine content of the powder from substantially .5% up to .65%; and using 80% alcohol containing 19 pounds of diphenylamine per 10,000 pounds of solution I have raised the diphenylamine content of the powder from substantially .5% up to .75%.

As previously indicated, the method may be applied particularly advantageously when used in conjunction with that method, for removing ethyl ether and ethyl alcohol solvent from nitrocellulose powder, which comprises first washing with ethyl alcohol to remove the ether, except for that corresponding to the desired residual solvent, draining the alcohol from the powder and then washing with water to remove the alcohol; for addition of the diphenylamine to the alcohol used for washing out the ether prevents the extraction of the diphenylamine contained in the powder. As examples of this use of the method in the retaining

of stabilizer, I have proceeded as described below, with satisfactory results:—

In washing "green" nitrocellulose powder with 60% alcohol, the powder containing substantially .5% of diphenylamine, i. e. 70 containing a weight of diphenylamine equal to substantially .5% of the weight of the corresponding "dry" or finished powder, 3 to 4 pounds of diphenylamine to each 10,000 pounds of solution gives the necessary equilibrium and preserves the diphenylamine content at substantially .5%.

In washing "green" powder containing substantially .5% of diphenylamine (dry powder basis) with 80% alcohol, 10 to 11 80 pounds of diphenylamine to each 10,000 pounds of solution gives the necessary equilibrium.

As previously stated, the method may be practiced with alcoholic solutions of other strengths. So far as I am aware the "curves" obtained by plotting "percentage of diphenylamine in the finished powder" against the corresponding experimentally determined values of "percent of diphenylamine in the alcohol", in the usual way, are straight lines. The formulas will be similar to those given above, the value of "B" being the percent at which the "curve" meets the "percent in powder" axis, shown 95 by the plot.

I claim:

1. The method of controlling the stabilizer content of a cellulosic colloid which comprises washing the colloid in a volatile 100 solvent containing the stabilizer.

2. The method of controlling the stabilizer content of a cellulosic colloid which comprises washing the colloid with a solution containing the stabilizer, and then 105 washing the colloid in a liquid in which the solvent of the stabilizer is miscible and the stabilizer is insoluble.

3. The method of controlling the stabilizer content of a stabilizer-containing cellulosic colloid during washing with a volatile 110 liquid in which the stabilizer is soluble, which comprises adding to the washing liquid an amount of stabilizer sufficient to give equilibrium between the colloid-contained 115 stabilizer and that in the washing liquid.

4. The method of controlling the stabilizer content of a stabilizer-containing cellulosic colloid during washing with a liquid 120 in which the stabilizer is soluble, which comprises adding to the washing liquid an amount of stabilizer in excess of that sufficient to give equilibrium between the colloid-contained stabilizer and that in the washing liquid, and then treating to remove 125 the washing liquid while leaving the stabilizer in the colloid.

5. The method of controlling the diphenylamine content of a cellulosic colloid during washing with ethyl alcohol which com- 130

prises adding diphenylamine to the alcohol.

6. The method of controlling the diphenylamine content of a cellulosic colloid which comprises washing with a substantially 60% solution of ethyl alcohol containing a percentage of diphenylamine determined in substantial accordance with the formula,—

$$10 \quad y = \frac{X - B}{4.5};$$

wherein X=per cent of diphenylamine desired in the finished powder, and B=per cent of diphenylamine already in the powder, this per cent B, for any values above 15 that percentage below which diphenylamine-free 60% alcohol will not reduce the diphenylamine content of the colloid, to be taken as that percentage.

20 7. The method of controlling the diphenylamine content of a cellulosic colloid which comprises washing with a substantially 60% solution of ethyl alcohol containing a percentage of diphenylamine determined in substantial accordance with the formula,—

$$25 \quad y = \frac{X - B}{4.5};$$

30 wherein X=per cent of diphenylamine desired in the finished powder, and B=per

cent of diphenylamine already in the powder, this per cent B, for any values above .37, to be taken as .37.

8. The method of controlling the diphenylamine content of a cellulosic colloid during washing with substantially 60% ethyl alcohol, which comprises adding diphenylamine to the alcohol in substantially the proportion of 3 to 4 pounds of diphenylamine to 10,000 pounds of alcohol.

9. The method of recovering ethyl alcohol and ethyl ether solvent from a nitrocelulose colloid containing a stabilizer soluble in ethyl alcohol, which comprises washing the colloid with ethyl alcohol containing stabilizer until the ether is sufficiently removed, draining alcohol from the colloid and then washing with water.

10. The method of removing ethyl alcohol and ethyl ether solvent from a nitrocelulose colloid containing substantially .5% of diphenylamine, which comprises washing the colloid in substantially 60% ethyl alcohol containing diphenylamine in substantially the proportion of 3 to 4 pounds of diphenylamine to 10,000 pounds of alcohol, until the ether is sufficiently removed, draining alcohol from the colloid and then washing with water.

35 45 50 55 60  
In testimony whereof I affix my signature.  
GEORGE ROCKER.